

# United States Patent Office.

THOMAS H. JENKINS, OF NYACK, NEW YORK.

*Letters Patent No. 67,121, dated July 23, 1867.*

## IMPROVED PROCESS OF MAKING STEEL.

The Schedule referred to in these Letters Patent and making part of the same.

### TO ALL WHOM IT MAY CONCERN:

Be it known that I, THOMAS H. JENKINS, of Nyack, Rockland county, and State of New York, have invented a new and useful improvement in the Process of Making Steel; and I do hereby declare that the following is a full, clear, and exact description thereof.

My said invention consists in making steel by melting, in pots or crucibles, wrought iron in admixture with from about five to twelve per centum of cast iron, which has been purified by being immersed, while in a highly-heated state, in a liquid bath.

In working according to my said invention, I take crude cast iron and heat it to a high temperature, preferring what is called a cherry-red heat, and then plunge it in a bath which, by preference, consists of twenty-eight gallons of water, eight pounds of oil of vitriol, forty-four ounces of sal-ammoniac, twenty ounces of Glauber salts, and thirty ounces of common table salt.

Other and equivalent solutions may be substituted. It will be found best to treat the iron in small pieces. After the crude cast iron has been thus treated, or purified, it is mixed with wrought iron, such as scrap iron, in the proportion of about from five to twelve per cent. of the purified cast iron, and in admixture melted in pots or crucibles, in the manner heretofore usually practised in the manufacture of cast steel.

I have above stated that I use the purified cast iron in the proportion of about from five to twelve per cent., because I have found that within that range I am enabled to produce the various grades, from the lowest to the highest temper, five per cent. of the purified cast iron producing the lowest, and twelve per cent. the highest grade of steel.

By my said process I am enabled to produce good steel with less labor and at less expense than by any other known process.

What I claim as my invention, in the process of making steel, is—

Melting wrought iron in crucibles or pots, in admixture with a percentage of crude cast iron, after such crude cast iron has been treated, while in a highly-heated state, in a bath, substantially as described.

THO. H. JENKINS.

Witnesses:

OSCAR BLAUVELT,

ANDREW A. DEMAREST.